

# UNITED STATES PATENT OFFICE.

JAMES NAULTY AND JOHN SCANLIN, OF PHILADELPHIA, PENNSYLVANIA.

## PROCESS OF MAKING COPPER ALLOYS AND THE PRODUCT THEREOF.

974,419.

Specification of Letters Patent.

Patented Nov. 1, 1910.

No Drawing.

Application filed July 23, 1910. Serial No. 573,525.

*To all whom it may concern:*

Be it known that we, JAMES NAULTY and JOHN SCANLIN, citizens of the United States, residing in the city of Philadelphia, 5 State of Pennsylvania, have jointly invented certain new and useful Improvements in Processes of Making Copper Alloys and the Products Thereof, of which the following is a full, clear, and exact description, reference 10 being had to the accompanying drawings, forming a part of this specification.

Our invention relates to a process of making chromium alloys of copper, compounded with nickel and other metals, and to the new 15 composition metal which is the product thereof, and has for its object to produce a copper alloy which is of great tensile strength and incidentally of sufficient hardness, approximately that of ordinary steel, 20 to made edged tools therefrom; and is well adapted for rolling, welding and forge work.

To these ends the invention consists of a particular method of compounding the elements of the composition, and the product thereof which is copper or its natural alloys combined with chromium and nickel, and with a relatively small proportion of aluminum and of zinc. The resultant composition 25 is essentially a copper alloy in which the chromium element is melted with the copper in approximately the ratio of five parts by weight of the former to one hundred and ten parts by weight of the latter; also in 30 which approximately twenty-five parts by weight, of nickel, to one hundred and ten parts of copper, are combined in the crucible; these elements, in or about the proportions stated being employed with twenty- 35 five parts by weight, in the aggregate, of zinc and aluminum, as hereinafter stated.

In carrying out the process to produce the new alloy, from the elements and in the quantitative ratios stated, five pounds of chromium are melted in a crucible with five pounds of aluminum of commerce, used as a flux, and which, with natural draft, will occupy about one hour, whereupon one hundred and ten pounds of copper are added to the mass in the crucible and melted, under a continued application of the same heat for about thirty minutes; after which twenty-

five pounds of nickel are placed in the crucible and which will combine with the other elements, in a molten mass in about one 55 hour; and finally twenty pounds of zinc are added, which melts almost instantaneously, and is employed principally for bulk or body purposes. Although the ratio stated of chromium to copper and of nickel to 60 copper are approximate only and may be slightly varied, the order stated in which the elements are admixed in the crucible, and the employment of aluminum as a flux, with the chromium, are essential; and finally it 65 must be understood that our new composition metal is essentially a copper alloy. It has a slightly reddish tinge, and tests of it, made from the formula above given, showed a tensile strength of 78950 pounds. In both 70 these respects it differs materially from the composition metal of copper and chromium combined with nickel and zinc, described in U. S. Patent No. 959,156 granted to us May 24, 1910, in which the large proportion of 75 nickel gives predominating color and characteristic to the composition, with perhaps greater hardness than our present alloy, but with decidedly less tensile strength, tests of it showing but 45000 pounds approxi- 80 mately.

Having thus described our invention, we claim as new and desire to secure by Letters Patent:—

1. The process of compounding a chromium alloy of copper, combined with nickel, which consists in melting the chromium with aluminum as a flux, then adding the copper, nickel and a suitable bulking metal to the molten mass successively and in the order 85 stated.

2. The product of the process described which is approximately a five per cent. chromium alloy of copper, combined with nickel in the ratio of approximately five parts by 90 weight of said copper alloy to one part by weight of nickel.

3. The new product described which is approximately a five per cent. chromium alloy of copper fluxed with aluminum, combined with nickel in the ratio of approximately five parts by weight of said copper alloy to one part by weight of nickel. 100

4. The new products described which is

approximately a five per cent. chromium alloy of copper fluxed with aluminum, combined with nickel and zinc in the ratio, in the aggregate, of approximately one hundred and twenty pounds of said copper alloy to forty-five pounds, in the aggregate, of nickel and zinc.

In testimony whereof, we have hereunto

affixed our signatures this twenty-first day of July A. D. 1910.

JAMES NAULTY.  
JOHN SCANLIN.

Witnesses:

A. M. BIDDLE,  
R. A. DUNLAP.